

# UNITED STATES PATENT OFFICE.

JAMES M. MASSON, OF DULUTH, MINNESOTA.

## METHOD OF AND BATH FOR RETTING FIBROUS STRAW.

1,374,941.

Specification of Letters Patent. Patented Apr. 19, 1921.

No Drawing.

Application filed January 12, 1920. Serial No. 350,978.

To all whom it may concern:

Be it known that I, JAMES M. MASSON, a citizen of the United States, residing at Duluth, in the county of St. Louis and State 5 of Minnesota, have invented certain new and useful Improvements in Methods of and Baths for Retting Fibrous Straw, of which the following is a specification.

My invention relates to the treatment of 0 flax or other straw in the art of producing fiber therefrom and which method is commonly known as tank retting and the process herein described is applicable to either flax or other fibrous straw as it comes from a 15 threshing machine, or to that which has been pulled especially for the purpose of fiber production.

This improved method involves the use of 20 a formula comprising certain solvent oils and mild alkalis which act quickly on the gum or resin and coloring matter in the straw, thoroughly dissolving all the former and bleaching both the straw and the fiber leaving the latter lustrous and soft without 25 impairing its quality. The fiber being entirely freed from gum or resin is readily separated from the shives which being well retted are easily crushed and removed from the fiber by the succeeding processes of de- 30 corticating et cetera.

Heretofore all known methods of tank retting of fibrous straw has been accomplished by the use of strong caustic alkalis and prolonged treatment which is well 35 known to those versed in the art to be a serious handicap in the economical production of fiber, and to overcome which is the principal object of my present invention, together with the production of a better, 40 brighter and more silky fiber than heretofore known.

Other objects and advantages of the improved method and formula for use therein 45 will appear in the further description of the invention.

The formula or composition of the bath employed comprises: one fluid ounce per gallon of a sulfonated castor oil, (sometimes known as turkey-red oil) or other similar 50 oils, one ounce avoirdupois pure alkali, (known as solvay alkali) and one ounce avoirdupois per gallon of tri-phosphate of soda.

The desired quantity of this solution is 55 placed within a suitable tank, the straw

placed therein and the composition heated and brought to boiling point, said boiling maintained for approximately 30 to 40 minutes when it is then allowed to steep for 2 or 3 hours. Then the straw and fiber are 60 removed and thoroughly washed in hot water to which has been added a small amount of ammonia for the thorough washing away of the dissolved gums.

Then the retted straw is removed and all 65 water with residue extracted by centrifugal or other suitable process, when it is thoroughly dried at a moderate temperature either by natural or artificial heat.

Having thus described my invention, what 70 I claim as new and desire to secure by Letters Patent is:

1. The method herein described of retting fibrous straw consisting in submerging and boiling the straw in a solution containing 75 tri-phosphate of soda and sulfonated oils, and subsequently removing and washing the straw.

2. The method herein described of retting fibrous straw consisting in submerging and 80 boiling the straw in a solution containing tri-phosphate of soda and sulfonated oils, and subsequently removing and washing the straw in hot water to which ammonia has been added.

3. The method herein described of retting fibrous straw in a solution composed of one fluid ounce per gallon of sulfonated castor oil, one ounce avoirdupois pure alkali, and one ounce avoirdupois tri-phosphate of 90 soda, and subsequently removing the straw and washing it for further treatment.

4. The method herein described of retting fibrous straw in a solution composed of one fluid ounce per gallon of sulfonated oils, one 95 ounce avoirdupois pure alkali and one ounce avoirdupois tri-phosphate of soda, and subsequently washing same for further treatment.

5. The method herein described of tank 100 retting fibrous straw consisting in boiling and steeping the straw in a solution containing sulfonated oils, alkali and tri-phosphate of soda, then removing the straw from such solution and washing same for subsequent 105 treatment.

6. The method herein described of tank retting fibrous straw consisting in boiling and steeping the straw in a solution containing sulfonated oils, alkali and tri-phosphate of 110

soda, then removing the straw from such solution and washing same in hot water to which ammonia has been added.

7. A bath for tank retting of fibrous straw comprising sulfonated castor oil, pure alkali and tri-phosphate of soda.

8. A bath for tank retting of fibrous straw composed of one fluid ounce per gallon of a sulfonated castor oil, one ounce avoirdupois

pure alkali and one ounce avoirdupois of 10 tri-phosphate of soda, substantially as described.

In testimony whereof I hereunto affix my signature in the presence of two witnesses.

JAMES M. MASSON.

Witnesses:

M. L. EVJEN,  
S. GEO. STEVENS.